



US005916405A

# United States Patent [19]

Ritto et al.

[11] Patent Number: **5,916,405**[45] Date of Patent: **\*Jun. 29, 1999**[54] **LIGHTWEIGHT SPEAKER ENCLOSURE**[75] Inventors: **Ross Ritto**, Encinitas; **Michael Adams**, Vista, both of Calif.[73] Assignee: **Southern California Sound Image, Inc.**, Escondido, Calif.

[\*] Notice: This patent issued on a continued prosecution application filed under 37 CFR 1.53(d), and is subject to the twenty year patent term provisions of 35 U.S.C. 154(a)(2).

[21] Appl. No.: **08/600,310**[22] Filed: **Feb. 12, 1996****Related U.S. Application Data**

[62] Division of application No. 08/303,947, Sep. 9, 1994, Pat. No. 5,519,178.

[51] **Int. Cl.<sup>6</sup>** ..... **A47B 81/06**; B32B 31/04[52] **U.S. Cl.** ..... **156/245**; 156/285; 181/199; 264/258[58] **Field of Search** ..... 156/245, 285, 156/286, 307.3; 264/257, 258; 181/148, 151, 199, 290, 292[56] **References Cited****U.S. PATENT DOCUMENTS**

|           |         |                |         |
|-----------|---------|----------------|---------|
| 1,965,830 | 7/1934  | Hammer         | .       |
| 2,670,053 | 2/1954  | Doms           | .       |
| 3,804,195 | 4/1974  | Everitt et al. | 181/148 |
| 3,985,201 | 10/1976 | Kloster        | .       |
| 4,042,778 | 8/1977  | Clinton        | 381/182 |
| 4,071,111 | 1/1978  | Croup          | 181/149 |

|           |         |                   |         |
|-----------|---------|-------------------|---------|
| 4,109,983 | 8/1978  | Kinoshita         | .       |
| 4,284,168 | 8/1981  | Gaus              | .       |
| 4,596,305 | 6/1986  | Jagborn           | 181/199 |
| 4,811,403 | 3/1989  | Henricksen et al. | 381/87  |
| 4,905,860 | 3/1990  | Kurihara          | 381/86  |
| 4,957,184 | 9/1990  | Negishi           | 181/199 |
| 4,964,482 | 10/1990 | Meyer             | 181/199 |
| 5,067,583 | 11/1991 | Hathaway          | 181/151 |
| 5,168,129 | 12/1992 | D'Antonio         | .       |

**FOREIGN PATENT DOCUMENTS**

191995 10/1984 Japan .

*Primary Examiner*—Daniel Stemmer*Attorney, Agent, or Firm*—Knobbe, Martens, Olsen & Bear, LLP

[57]

**ABSTRACT**

A speaker enclosure having a substantially seamless rigid outer skin, a middle sound absorbing layer, and a substantially seamless flexible inner skin. The speaker enclosure is comprised of two basic parts, a box section and a baffle section where each of these sections include the rigid outer skin, the middle sound absorbing layer and the seamless flexible inner skin and are made according to the same method. The outer skin is formed from multiple layers of resin impregnated carbon fiber, the middle sound absorbing layer includes pieces of honeycomb material and the inner layer is formed from multiple layers of resin impregnated fiberglass. The layers of material are arranged in a substantially seamless manner into a mold and then cured by vacuum bagging and heating thereby producing a strong, lightweight speaker enclosure made of materials which dampen the transmission of errant sound waves in the enclosure and thereby minimize distortion of the sound signal produced by the speaker.

**25 Claims, 4 Drawing Sheets**



Figure 1

**Figure 2**

**Figure 3**



**Figure 5**



**Figure 4**

**LIGHTWEIGHT SPEAKER ENCLOSURE**

This application is a divisional of U.S. patent application Ser. No. 08/303,947, filed Sep. 9, 1994, now U.S. Pat. No. 5,519,178.

**BACKGROUND OF THE INVENTION****FIELD OF THE INVENTION**

The present invention relates to an improved speaker enclosure and, in particular, concerns a speaker enclosure seamlessly manufactured out of lightweight, sound absorbing materials.

**DESCRIPTION OF THE RELATED ART**

Speaker enclosures of the prior art are typically made out of a semi-rigid material, such as plywood, and have a box-like shape. The front side of the speaker enclosure includes a baffle which has several openings in which the diaphragm portion of the speaker is positioned so that sound can emanate out from the speaker enclosure. This describes the typical speaker enclosure that is used in many different applications including speakers for home use and speakers for use at music concerts.

One difficulty that occurs in many large prior art speaker enclosures is that they are very heavy. In particular, the large speakers that are used, for example, in music concerts require large speaker enclosures. Generally, the enclosures have to be made out of fairly thick material to support the weight of the speakers. Consequently, speaker enclosures can become very heavy. As can be appreciated, the heavier the speaker enclosure, the more difficult it is to move and support the speaker enclosure. In some instances, the increased weight results in difficulties in mounting these enclosures.

For example, it is often desirable to mount speakers over the heads of the performers and audience at musical concerts. However, heavy speaker enclosures pose a risk of the speaker enclosures breaking loose from their supports and falling on the performers or the audience. To minimize this risk, heavy duty supports are needed to securely retain the speaker enclosures. It can be appreciated, however, that these supports increase the cost of installing the speaker enclosures and can also increase the time required to mount the enclosures.

A further difficulty that results from constructing speaker enclosures out of materials such as plywood is that these materials often degrade the sound performance of the speaker. Ideally, all of the sound that is produced by the speaker should emanate outward from the diaphragm of the speaker away from the speaker enclosure. However, there are typically some errant sound waves which travel inward into the speaker enclosure.

A semi-rigid material, such as plywood, has a tendency to vibrate in response to these inwardly travelling errant sound waves. These vibrations can result in distortion of the sound produced by the speakers. To minimize these vibrations, sound engineers often have to place materials inside of the speaker enclosure to dampen the errant sound waves and minimize the vibrations. However, the speaker enclosures are typically configured so as to maximize the output of the speakers and placing extraneous materials and objects inside the speaker enclosures can further result in degradation of the sound performance of speaker.

To address these problems, some speaker enclosure designers have built enclosures for speakers out of materials

that are lightweight and could, conceivably, absorb some errant sound waves. One example of such an enclosure is shown in U.S. Pat. No. 3,804,195 which discloses a loudspeaker enclosure made out of corrugated sheets of material.

5 The corrugated sheets of material include hollow portions. Each of these sheets are joined to each other in a box-like configuration. Another example is U.S. Pat. No. 4,811,403 which discloses a lightweight loudspeaker enclosure that uses a rigid lightweight honeycombed material in part of the speaker enclosure.

10 While the weight characteristics and sound performance of the speaker enclosure disclosed in the U.S. Pat. No. 3,804,195 and the U.S. Pat. No. 4,811,403 may be improved by the use of the corrugated material, there will still be vibrations of the speaker enclosure due to the fact that there are seams which join each of the pieces of the enclosure. The errant sound waves induce vibrations at the seams and joints between the individual materials and thereby reduce the overall sound performance or efficiency of the speakers. 15 Further, the enclosures disclosed in both these patents still have some surfaces and materials which vibrate in response to errant sound waves and thereby reduce the overall efficiency and sound performance of the speakers.

20 Hence, there is a need in the art for a lightweight speaker enclosure which minimizes distortion of the sound signal produced by the speakers as a result of errant sound waves in the speaker enclosure. To this end, there is a need for a speaker enclosure that is made out of a composite of strong lightweight materials that have sound absorbing qualities. 25 Further, this speaker enclosure should also be as seamless as possible to minimize the sources of distortion of the sound signals.

**SUMMARY OF THE INVENTION**

30 The aforementioned needs are satisfied by the sound speaker enclosure of the present invention which generally includes a box section formed of an outer skin of a rigid material, a middle layer of a sound absorbing material, and an inner skin of a flexible material and a baffle section that includes the same three layer construction. The baffle section is then preferably bonded to the box section of the speaker enclosure to thereby complete the speaker enclosure.

35 In one aspect of the present invention, the box section and the baffle section of the speaker enclosure are constructed so that there are virtually no seams between different walls of the enclosure. In the preferred embodiment this is accomplished by individually constructing the box and baffle section of the speaker enclosure out of generally flexible overlapping pieces of material that are then cured into a rigid or semi-rigid state. Once both the box and baffle section of 40 the speaker enclosure are constructed, they are then bonded to each other in a virtually seamless bond.

45 In another aspect of the present invention, the rigid outer skin of the speaker enclosure is made out of a material that, when cured, is very hard. This hard outer skin minimizes the likelihood of the enclosure vibrating due to errant sound waves. In the preferred embodiment, the rigid outer skin is made of overlapping layers of a carbon fiber material.

50 In yet another aspect of the present invention, the middle layer includes air pockets which are designed to trap the errant sound waves in the interior of the speaker enclosure to prevent their reflection and retransmission. In the preferred embodiment, the middle layer is made of pieces of honeycomb material sold under the trademark Nomex that includes air pockets which can absorb sound waves.

55 In yet another aspect of the present invention, the inner flexible skin is made of a skin that is sufficiently flexible to

absorb, and not reflect, the errant sound waves. In the preferred embodiment, the inner flexible skin is made of overlapping layers of fiberglass that are cured into a hardened, yet flexible, state.

Thus, the present invention discloses a sound speaker enclosure which has a box section and a baffle section where both sections are virtually seamless, are manufactured out of lightweight yet strong materials and are designed to maximize the performance of the sound speakers by minimizing both retransmission of errant sound waves and vibrations resulting from these errant sound waves. These and other objects and features of the present invention will become more fully apparent from the following description and appended claims taken in conjunction with the accompanying drawings.

#### BRIEF DESCRIPTION OF THE DRAWINGS

FIG. 1 is a perspective view of the speaker enclosure of the present invention which is partially cut away to illustrate the layers of material comprising the walls of the speaker enclosure;

FIG. 2 is an exploded perspective view of a section of one of the walls of the speaker enclosure of FIG. 1 which illustrates the layers of the speaker enclosure in greater detail;

FIG. 3 is a partial perspective view of a section of two of the walls of the speaker enclosure, taken along lines 3—3 of FIG. 1, which further illustrates the organization of the layers of material forming the walls of the speaker enclosure;

FIG. 4 is an exploded side view of a circled section of two of the walls of the speaker enclosure shown in FIG. 3 which further illustrate the organization of the layers of material forming the walls of the speaker enclosure; and

FIG. 5 is a perspective view of a male mold used to fabricate the baffle section of the speaker enclosure shown in FIG. 1.

#### DESCRIPTION OF THE PREFERRED EMBODIMENTS

Reference will now be made to the drawings wherein like numerals refer to like parts. FIG. 1 illustrates a speaker enclosure 100 of the present invention. The speaker enclosure 100 in this preferred embodiment is comprised of two basic component parts, a box section 102 and a baffle section 104. The box section 102 defines a volume of enclosed space in which one or more speakers 106 (shown in phantom) are positioned. In the embodiment of the speaker enclosure 100 shown in FIG. 1, the box section 102 is shown to have a generally rectangular shape with two back walls 108 that are flanged outwardly from a front face 110 of the box section 102.

The baffle section 104 includes one or more openings 112 where the speakers 106 are mounted so that the diaphragm portion of the speakers communicate through the openings 112 to the outside of the speaker enclosure 100. The baffle section 104 is dimensioned to rest on a ledge 114 which extends around the inside perimeter of the front face 110 of the box section 102 of the enclosure 100. In this preferred embodiment, the ledge 114 is preferably dimensioned to allow the baffle section 104 to rest flush with front face 110 of the box section 102. The ledge 114 is also preferably made of a material such as styrofoam which provides a surface whereby the baffle section 104 can be securely bonded to the box section 102.

It should be appreciated that the speaker enclosure 100 can be any of a number of shapes and sizes depending upon the desired use of the speaker enclosure. Hence, the following description of the construction of the speaker enclosure 100 of the present invention is readily adaptable to any size and shape of speaker enclosure and is not limited to the exact enclosure shown in these figures.

The cut away section of FIG. 1 also illustrates that the walls of the box section 102 are comprised of a plurality of layers of material generally indicated by the reference numeral 116. The speaker enclosure 100 of the present invention is advantageously constructed of a plurality of layers of materials which are positioned in a mold 120 in a layered fashion and then cured in the manner described below. The mold 120 is, in this preferred embodiment, a female wood mold which has the exact dimensions and configuration as the outside of the box section 102 of speaker enclosure 100. The mold 120 is hand made to the exact tolerances desired and then sanded to allow for easy removal of the box section 102 after fabrication.

The layers that are positioned in the mold 120 to produce the walls of the box section 102 of the sound enclosure 100 will now be described by reference to FIG. 2. FIG. 2 is an exploded perspective view of the of the layers 116 that comprise both the walls of the box section 102 of the enclosure 100 and the wall of the baffle section 104. These layers 116 are positioned in the mold 120 and are then vacuum bagged and cured using conventional techniques that are described in greater detail below.

Generally, the mold 120 is initially coated with one or more release agents to permit easy removal of the speaker enclosure 100 from the mold 120 once the layers 116 have been cured. In this preferred embodiment, the inner surface of the mold 120 is thoroughly coated with three coats of FREAKOUT 700-NC release agent manufactured by Freakout Co. of Seabrook, N.H., three coats of PA0801 Flourotolomer Wax Dispersion manufactured by PTM & W Industries of Santa Fe Springs Calif. and one coat of E-91 N-ODS monocoat material manufactured by Chem Trend Inc. of Howell, Mich.

Once the release agent is applied to the mold 120, the first of the layers 116 is then positioned inside of the mold 120. Specifically, three layers of flexible material 122a, 122b and 122c that cures into a hardened material are positioned inside of the mold. In this preferred embodiment, the material 122 is a carbon fiber material that is a flexible cloth material impregnated with resin. Each layer of material 122 is comprised of a plurality of pieces of the fabric that are cut and then positioned inside of the mold 120. The plurality of pieces are cut to size to fit the various walls of the box enclosure 102 or the baffle section 104 and these pieces comprising the layers 116 are preferably cut so as to overlap at the borders between two walls of the box section 102 as is shown in greater detail in FIGS. 3 and 4.

Preferably, the carbon fiber layers 122a, 122b and 122c are made of three alternating weaves of carbon fiber to provide additional strength to the outer surface of the box 102 once the layers 116 have cured. Specifically, in this preferred embodiment, the three carbon layers 122a-122c are comprised of a layer having a 0/90 weave, a layer having a +/-45 weave and a layer having a 0/90 weave respectively. Further, in this preferred embodiment, each of these layers 122 are preferably comprised of series 282 Carbon Fiber Prepreg cloth with a 40% resin content wherein the resin cures at 250° F. Carbon fiber meeting these requirements is available from JD Lincoln Co. in Costa Mesa, Calif.

Once each of the layers 122 are positioned in the mold 120, and a layer of film adhesive 124 is then positioned over the layer of carbon fiber 122c. The layer of film adhesive 124 is comprised of a thin layer of cloth that contains resin which allows pieces of a sound absorbing material 126 to adhere to the carbon fibers 122 upon curing.

Once the layer of film adhesive 124 is positioned inside of the mold 120, a plurality of pre-cut pieces of sound absorbing material 126 are then positioned inside of the mold 120 on top of the film adhesive 124. Preferably, the sound absorbing material 126 is comprised of a material which defines a plurality of air pockets that are capable of absorbing sound waves produced by the speaker 106. In this preferred embodiment, the sound absorbing material 126 is comprised of Nomex brand material. Nomex is a brand name of a material manufactured by Dupont that is essentially comprised of a paper base impregnated with resin, to give rigidity to the material, that forms a plurality of open cells. In this preferred embodiment, Nomex brand material having a 4.8 pound density with  $\frac{1}{4}$ " cells and that is available as AHN 4120 Nomex Honeycomb from Advanced Honeycomb Inc. of San Marcos, Calif., is used.

In this preferred embodiment, the sound absorbing material 126 is rigid so it can't be laid into the mold 120 in an overlapping fashion. Hence, the sound absorbing material 126 has to be cut into a plurality of pieces which are preferably configured so that as much as possible of the surface of the inner walls of the box section 102 is covered with the sound absorbing material 126. As can be appreciated, the exact dimensions of the pieces of sound absorbing materials 126 depend upon the configuration of the speaker enclosure 100, which can vary depending upon the desired shape and use of the enclosure.

Once the plurality of pieces of sound absorbing material 126 have been positioned in the mold 120, pieces of film adhesive, forming two layers of film adhesive 128a and 128b are then positioned on top of the layer of sound absorbing material 126. The layers of film adhesive 126 bond the sound absorbing material 126 to three layers of flexible material 130a-130c. The three layers of flexible material 130a-130c, in this preferred embodiment, are comprised of schedule 7781 E-glass which is a type of fiberglass. Preferably, the flexible material 130 used in the present invention is flexible and can be laid on the layer of film adhesive 128 in the same manner as a layer of cloth. Hence, pieces of the material 130 are cut to fit each section of the walls of the enclosure 100. Preferably, these pieces comprising the layers are cut so that, at the intersection between two walls, there is an overlap of the material 130.

A layer of release fabric 132, a layer of perforated release film 134 and a layer of air weave material 136 are then preferably positioned on top of the layers of the flexible semi-rigid material 130. The layer of release film 134 and air weave material 136 are preferably positioned over the front face 110 of the box section 102 of the enclosure 100 and are firmly attached at their periphery to the mold 120. These layers allow excess resins and volatiles to escape from the layers of carbon, sound absorbing material and E-glass upon curing of the box section 102 of the enclosure 100.

Once each of these layers is positioned inside the mold 120, a vacuum bag (not shown) is positioned on top of the mold 120 to thereby allow the resins and layers of material to cure by vacuum bagging in a manner well known in the art. Specifically, in the preferred embodiment of the present invention, an assembled mold comprising the mold 120 with the layers 116 is vacuum cured over a given temperature

range for approximately 2 hours at -85kPa, -25 in Hg pressure. Preferably, the assembled mold is initially positioned in an oven which is heated to approximately 140-160° F. Once the assembled mold attains this temperature, the oven is then heated to 250° F. at a rate of approximately 1° per minute. The assembled mold then cures at this temperature for 2 hours after which the oven cools at a rate no faster than 4° F. per minute.

The curing process results in curing and hardening of the 10 resins contained in the carbon fiber layers 122, the film adhesive layers 124 and 128 and the layers of flexible material 130. Consequently, after the curing process, the walls of the enclosure 100 are then comprised of three basic layers of material, a rigid outer skin 122', a layer of sound 15 absorbing material 126' and a flexible inner skin 130'.

The rigid outer skin 122' is comprised of the three hardened layers of carbon fiber 122a-122c. Preferably the rigid outer skin 122' is sufficiently strong so as to both minimize the tendency of the box section 102 of the enclosure 100 to vibrate in response to errant sound waves produced by the speaker 106 and to prevent the escape of 20 these sound waves through the walls of the box section 102 of the enclosure. As can be appreciated, the rigid outer skin 122' can be made of a number of different materials that will 25 cure into a hardened rigid material including other carbon materials, Kevlar etc.

The flexible inner skin 130' is thus comprised of the three 30 cured layers of fiberglass 130a-130c. The inner skin 130' is preferably sufficiently flexible to vibrate in response to the errant sound waves inside the speaker enclosure 100 and thereby absorb and not reflect these sound waves. As can be appreciated, the inner flexible skin 130' can be made of any 35 material which has sufficient flexibility upon final assembly of the enclosure 100 to minimize reflection of these errant sound waves. Since the pieces of material forming the rigid outer skin 122' and the flexible inner skin 130' overlap at the junction between the walls, the box portion 102 of the enclosure is formed with virtually no seams between walls. This overlapping of the pieces comprising the layers of 40 material is more clearly illustrated in FIGS. 3 and 4. In both FIGS. 3 and 4, junctions between two walls of the mold 120, and thus junctions between two walls of the box section 102 of the enclosure, have overlapping pieces of the carbon fiber 122 and the fiberglass 130. Further, the excess resins in the 45 various layers 116 seep into the spaces 140 between the pieces of sound absorbing material 126 forming the sound absorbing material layer 126'. Consequently, the layer of sound absorbing material 126' is also a substantially 50 continuous, seamless layer throughout entire box section 102 of the enclosure 100.

The seamless nature of the box section 102 of the enclosure 100 ensures that one wall of the box section 102 of the enclosure does not flex relative to another wall of the enclosure 100 as a result of errant sound waves impinging upon the walls. This results in less vibration of the enclosure 100 and minimizes the amount of errant sound waves escaping from the back and sides of the enclosure 100. Consequently, there is less distortion of the sound signal 55 generated from the speakers 106 mounted in the speaker enclosure 100 of the present invention.

Furthermore, the structure of the walls of the box, i.e., being comprised of a rigid outer skin 126', a layer of sound absorbing material 126' and an flexible inner skin 130' also 60 results in less distortion of the sound signal produced by the speakers 106. Specifically, the rigid outer skin 122' in this preferred embodiment is significantly more rigid than other 65

materials used in the construction of speaker enclosure such as plywood. Consequently, the speaker enclosure **100** as a whole does not vibrate in response to errant sound waves to the degree that a prior art speaker enclosure made of plywood.

However, the inner layer of flexible inner skin **130'** acts so as to absorb errant sound waves by flexing in response to the errant sound waves. Further, the middle sound absorbing layer **126'** acts as a chamber, in a manner analogous to the chamber created by double wall construction in sound studios, to trap the sound waves absorbed by the flexible inner skin **130'**.

The foregoing description has presented a method of fabricating the box section **102** of the speaker enclosure **100**. In this preferred embodiment, the baffle section **104** is also fabricated using a suitable male mold and according to the above-described method with the above-described materials. Referring now to FIG. 5, a sample male mold **150** used to fabricate the baffle section **104** is shown. The mold **150** includes a plurality of raised surfaces **152** at the position of the openings **110** in the baffle section **104**. Further, the mold **150** has a lip **154** around the perimeter of the mold **150** which projects outward from the surface of the mold **150** a distance sufficient to retain the layers **116** inside of the mold **150** during fabrication. As can be appreciated, the exact shape and configuration of the mold **150** and the pieces of materials forming the layers **116** depends upon the desired shape and configuration of the baffle section **104**.

Hence, in this preferred embodiment, the baffle section **104** is fabricated from cut overlapping pieces of carbon fiber **122** forming the original outer skin **122'**, cut pieces of sound absorbing material **126** forming the middle sound absorbing layer **126'** and cut overlapping pieces of fiberglass **130** forming the inner flexible skin **130'** in the same manner as the box section **102** described above. Consequently, the baffle section **104** is preferably made of the same materials as the box section **102** and, thus, has the same advantages in weight and strength and absorption of the errant sound waves.

Thus, the enclosure **100** of the present invention is comprised of a seamless box section **102** and a baffle section **104** that have the above-described sound absorbing capabilities. The only seam in the entire enclosure **100** is the seam between the box section **102** and the baffle section **104**. As described above in reference to FIG. 1, the baffle section **104** preferably is flushly positioned on the ledge **114** in the box section **102**. In this preferred embodiment, the ledge **114** is formed from pieces of Klegicell brand foam manufactured by Barracuda Technologies Inc. of Desoto, Tex. which are bonded to the perimeter of the front face **110** of the box section **102** and also to the baffle section **104** of the enclosure **100**. In this preferred embodiment the foam ledge **114** is bonded to both the box section **102** and the baffle section **104** of the enclosure using RF 912/130 two part epoxy from Resin Formulators Co. of Culver City, Calif.

Thus, the present invention described herein comprises a sound speaker enclosure which is virtually seamless and is made of sound absorbing materials. Further, the materials used in the preferred embodiment of the speaker enclosure **100** described herein result in a speaker enclosure **100** that is significantly lighter yet stronger than comparably sized prior art speaker enclosures. Hence, the speaker enclosures of the present invention can be more readily mounted and supported in different positions than the heavier speaker enclosures of the prior art.

Although the foregoing description of the preferred embodiment of the present invention has shown, described

and pointed out the fundamental novel features of the invention, it will be understood that various omissions, substitutions, and changes in the form of the detail of the apparatus as illustrated, as well as the uses thereof, may be made by those skilled in the art, without departing from the spirit of the present invention. Consequently, the scope of the invention should not be limited to the foregoing discussion, but should be defined by the appended claims.

What is claimed is:

1. A method of manufacturing a speaker enclosure comprising the steps of:  
 positioning a resin impregnated carbon fiber material into a female mold configured to form a box section of said speaker enclosure so that said resin impregnated carbon fiber material forms a continuous substantially seamless layer;  
 positioning a sound absorbing material in said female mold on top of said seamless layer of said carbon fiber material;  
 positioning a fiberglass resin impregnated material in said female mold on top of said sound absorbing material so that said fiberglass resin impregnated material forms a continuous substantially seamless layer;  
 curing said box section of said speaker enclosure so that said carbon fiber layer of material forms a substantially seamless rigid outer skin of said speaker enclosure, and said fiberglass layer of material forms a substantially seamless flexible inner skin of said enclosure with said layer of sound absorbing material interposed therebetween; and  
 attaching a baffle section to said box section which is formed after said curing step, wherein said baffle section includes an opening for a diaphragm of a speaker positioned inside said speaker enclosure defined by said box section and said baffle section.
2. The method of claim 1, wherein said step of positioning a resin impregnated carbon fiber material into a female mold comprises the steps of:  
 coating said mold with one or more release agents; and  
 positioning pieces of resin impregnated carbon fiber into said mold so that there are three superposed layers of resin impregnated carbon fiber in said mold and wherein said three layers of resin impregnated carbon fibers respectively have weaves of 0/90, +/−45 and 0/90.
3. The method of claim 2, wherein the step of positioning a sound absorbing material in said female mold comprises the steps of:  
 positioning a layer of film adhesive on the top layer of said layers of carbon fiber; and  
 positioning a plurality of pieces of honeycomb material on said layer of film adhesive.
4. The method of claim 3, wherein said honeycomb material comprises cells of approximately  $\frac{1}{4}$ " in cross section and has a density of approximately 4.8 Lbs.
5. The method of claim 3, wherein the step of positioning a fiberglass resin impregnated material into said female mold comprises the steps of:  
 positioning one or more layers of film adhesive onto said layer of sound absorbing material; and  
 positioning a plurality of pieces of resin impregnated fiberglass onto said layers of film adhesive such that said plurality of resin impregnated fiberglass pieces are arranged into a plurality of substantially seamless layers of resin impregnated fiberglass.

6. The method of claim 5, wherein said plurality of pieces of resin impregnated fiberglass are comprised of schedule 7781 E-glass.

7. The method of claim 5, wherein said step of curing said box section comprises the steps of:

- 5 positioning a layer of release fabric in said mold containing said layers of carbon fiber, sound absorbing material and fiberglass;
- positioning a layer of release film over said layer of release fabric;
- 10 positioning a layer of air weave over said layer of release film;
- vacuum bagging said mold containing said layers of carbon fiber, sound absorbing material and fiberglass; and
- 15 heating said mold containing said layers of carbon fiber, sound absorbing material and fiberglass.

8. The method of claim 7, wherein the step of heating said mold comprises the steps of:

- 20 pre-heating an oven to a temperature in the range of about 140 to 160 degrees Fahrenheit;
- positioning said mold into said oven;
- increasing said temperature in said oven to approximately 250 degrees Fahrenheit at a rate of increase of no more than about 1 degree per minute;
- 25 heating said mold in said oven at a temperature of 250 degrees Fahrenheit for approximately 2 hours; and
- cooling said mold to room temperature at a cooling rate of no more than about 4 degrees Fahrenheit per minute.

9. The method of claim 8, wherein the resin in said resin impregnated carbon fiber and in said fiberglass cures at about 250 degrees Fahrenheit.

10. The method of claim 1, further comprising the step of manufacturing said baffle section, wherein said manufacturing step comprises the steps of:

- 30 positioning a first resin impregnated material into a male mold configured to form a baffle section of said speaker enclosure so that said first resin impregnated material forms a continuous substantially seamless layer of said first material;
- positioning a sound absorbing material in said male mold on top of said substantially seamless layer of said first material;

- 35 positioning a second resin impregnated material into said male mold on top of said sound absorbing material so that said second resin impregnated material forms a continuous substantially seamless layer of said second material;

- 40 curing said baffle section of said speaker enclosure so that said first layer of material forms a substantially seamless rigid outer skin of said baffle section of said speaker enclosure, and said second layer of material forms a substantially seamless flexible inner skin of said material.

11. The method of claim 10, wherein said baffle section is bonded to a front face of said box section.

12. A method of making a speaker enclosure comprising the steps of:

- 45 positioning a resin impregnated carbon fiber material in a mold to form a continuous layer substantially covering an inner surface of said mold wherein the inner surface of said mold defines an outer surface of a box section of said speaker enclosure;

- 60 positioning a sound absorbing material into a cavity formed by said carbon fiber material positioned in said mold;

positioning a resin impregnated fiberglass layer in a cavity formed by said sound absorbing layer wherein the fiberglass layer, when cured, allows sound waves to travel therethrough to said sound absorbing material; curing said continuous layer of said carbon fiber material, and said fiberglass layer to form said box section of said speaker enclosure so that said box section comprises a substantially seamless outer skin of said carbon fiber material surrounding said sound absorbing material; and attaching a baffle section to said box section wherein said baffle section includes an opening for a diaphragm of a speaker positioned inside said speaker enclosure defined by said box section and said baffle section.

13. The method of claim 12, wherein the step of positioning a carbon fiber material in said mold comprises:

- positioning a first carbon fiber material having a first weave on the inner surface of said mold so as to form a first layer of carbon fiber material; and
- positioning a second carbon fiber material having a second weave on said first layer of carbon fiber material so as to form a second layer of carbon fiber material.

14. The method of claim 13, wherein the step of positioning a carbon fiber material in said mold comprises positioning a resin impregnated carbon fiber material in said mold.

15. The method of claim 12, wherein the step of positioning a carbon fiber material in said mold comprises the steps of:

- 30 positioning pieces of carbon fiber material into said mold so that there are three superposed layers of carbon fiber material covering said inner surface of said mold and wherein said three layers of carbon fiber material respectively have weaves of 0/90, +/-45 and 0/90.

16. The method of claim 12, wherein said sound absorbing material comprises a honeycomb material.

17. The method of claim 16, wherein said honeycomb material has a density of approximately 4.8 Lbs. and comprises cells of approximately 1/4" in cross section.

18. The method of claim 12, wherein said second layer of material comprises resin impregnated fiberglass material.

19. The method of claim 12, wherein said step of curing said box section comprises the steps of:

- 40 applying a vacuum to said mold containing said layer of carbon fiber material and said sound absorbing material; and

- 45 heating said mold containing said layer of carbon fiber material and said sound absorbing material.

20. A method of manufacturing a speaker enclosure comprising the steps of:

- 50 positioning one or more pieces of curable carbon fiber cloth material on a surface of a mold so that the carbon fiber cloth material forms a continuous layer covering the surface of said mold wherein the surface of said mold defines a surface of a box section of said speaker enclosure;

- 55 positioning one or more pieces of a sound absorbing material on a surface of said continuous layer of carbon fiber cloth material;

- 60 positioning a layer of resin impregnated fiberglass material adjacent said sound absorbing layer;

- 65 curing said continuous layer of carbon fiber cloth material, and said fiberglass layer so that said layer of carbon fiber cloth material forms a substantially seamless outer skin of said box section of said speaker

**11**

enclosure and said pieces of sound absorbing material are adhered to an inner surface of said substantially seamless outer skin and said fiberglass layer is adhered to an inner surface of said sound absorbing material; and

attaching a baffle section formed after said curing step to said box section wherein said baffle section includes an opening for a diaphragm of a speaker positioned inside said speaker enclosure defined by said box section and said baffle section.

**21.** The method of claim **20**, wherein said sound absorbing material comprises a honeycomb material.

**22.** A method of making a speaker enclosure comprising the steps of:

positioning a curable carbon fiber material in a mold so as to form continuous layer of carbon fiber material;

positioning a sound absorbing material in the mold;

positioning a layer of curable fiberglass material in the mold adjacent the sound absorbing material;

curing said carbon fiber material and said fiberglass material so that the carbon fiber material forms a substantially seamless outer skin of at least a portion of a box section of the speaker enclosure, said fiberglass layer forms an inner layer of said speaker enclosure that allows sound waves to pass therethrough and said sound absorbing material is interposed between the carbon fiber outer skin of the box section of the speaker enclosure and the inner layer of fiberglass material; and

5

10

20

25

attaching a baffle section to said box section which is formed after said curing step, wherein said baffle section includes an opening for a diaphragm of a speaker positioned inside said speaker enclosure defined by said box section and said baffle section.

**23.** The method of claim **22**, wherein the step of positioning a carbon fiber material in a mold comprises positioning a plurality of pieces of resin impregnated carbon fiber cloth material into said mold so that there are three superposed layers of resin impregnated carbon fiber cloth material in said mold wherein said three superposed layers of resin impregnated carbon fiber cloth material respectively have weaves of 0/90, +45 and 0/90.

**24.** The method of claim **22**, wherein the step of positioning sound absorbing material into a mold comprises positioning pieces of honeycomb material having a density of approximately 4.8 Lbs. and comprises cells of approximately  $\frac{1}{4}$ " cross section on an inner surface of the carbon fiber material.

**25.** The method of claim **22**, wherein the curing step is comprised of:

applying a vacuum to said mold containing said layer of carbon fiber material, said sound absorbing material and said fiberglass material; and

heating said mold containing said layer of carbon fiber material and said sound absorbing material.

\* \* \* \* \*